

May 4, 1948.

W. A. SISSON ET AL

2,440,761

APPARATUS FOR PRODUCING ARTIFICIAL FILAMENTS

Filed July 1, 1946

2 Sheets-Sheet 1



FIG. 1



FIG. 4



FIG. 2



FIG. 5



FIG. 3



FIG. 7



FIG. 6



FIG. 8



FIG. 9

INVENTORS.  
WAYNE A. SISSON  
WESLEY L. WEBB

BY *Carl A. Castellan*  
Attorney

May 4, 1948.

W. A. SISSON ET AL

2,440,761

APPARATUS FOR PRODUCING ARTIFICIAL FILAMENTS

Filed July 1, 1946

2 Sheets-Sheet 2



FIG. 2a



FIG. 3a



FIG. 3b

INVENTORS.  
WAYNE A. SISSON  
BY WESLEY L. WEBB

*Thomas R. O'Valley*

Patented May 4, 1948

2,440,761

# UNITED STATES PATENT OFFICE

2,440,761

## APPARATUS FOR PRODUCING ARTIFICIAL FILAMENTS

Wayne A. Sisson, Silverside Heights, Del., and Wesley L. Webb, Glen Moore, Pa., assignors to American Viscose Corporation, Wilmington, Del., a corporation of Delaware.

Application July 1, 1946, Serial No. 680,820

16 Claims. (Cl. 18—8)

1

This application is a continuation-in-part of our earlier copending application Serial No. 563,506, filed November 15, 1944, now abandoned which is in turn a division of our earlier copending application Serial No. 497,156, filed August 3, 1943 now Patent 2,428,046, September 30, 1947.

This invention relates to the production of filaments of composite character comprising at least two basic components, one of which is disposed between two portions of the other or others which may cover the lateral surfaces of the former component completely or only partially. In the former case, a core or sheath arrangement is obtained, while in the other, novel effects may be obtained.

It is an object of this invention to provide filaments having novel effects, and to provide apparatus for efficiently producing them alone or in combination with other filaments of different composition. Further objects and advantages of this invention will be apparent from the drawing and the description thereof hereinafter.

In the drawing illustrative of the invention— Figure 1 is a mid-section through an extrusion device constituting one embodiment of the invention,

Figure 2 is a cross-section taken on line II—II of Figure 1,

Figure 2a is a cross-section similar to Figure 2 of a modification,

Figure 3 is a cross-section taken on line III—III of Figure 1,

Figure 3a is a cross-section similar to Figure 3 of a modification,

Figure 3b is a cross-section similar to Figure 3 of another modification,

Figure 4 is a mid-section of another embodiment of the invention,

Figure 5 is a cross-section taken on line V—V of Figure 4,

Figure 6 is a cross-section taken on line VI—VI of Figure 4,

Figure 7 is a cross-section taken on line VII—VII of Figure 4,

Figure 8 illustrates in cross-section various of the novel filaments obtainable in accordance with the invention, and

Figure 9, illustrates in cross-section, additional varieties of filaments obtainable in accordance with the invention.

As shown in Figures 1 to 3, the spinneret 2 is attached to a supply head 3 for the spinning materials or solutions by a coupling 4. A gasket 5 is positioned between the flange of the spin-

2

neret 2 and the supply head 3 to assure a tight seal. Feed pipes 6 and 7 communicate with passages 8 and 9 respectively. Within the space back of the face of the spinneret 2, there is provided a partitioning means comprising a plate 10 from which a plurality of approximately parallel ribs 11 extend toward the back face of the spinneret without being in contact therewith. A partition 12 extends from the plate 10 in the opposite direction to divide the space back of the plate 10 into two separate regions A and B communicating with the passages 8 and 9 respectively. This partitioning means may be formed integrally within a cylindrical sleeve 13 fitting within the recess 14 within the supply head 3 and resting upon a spacing ring 15 to support the partitioning system out of contact with the back face of the spinneret. The spinneret is provided with two rows of orifices 16 arranged in registry with alternate spaces between the ribs 11. Thus, as is shown in Figure 3, every other space between the partitions 11 faces a portion of the spinneret face which is lacking in orifices, while the intervening spaces between partitions 11 are arranged in direct opposition to the spinneret orifices. Passages 17 through plate 10 connect the chamber B with the alternate spaces between ribs 11 which face blank portions of the spinneret, while passages 18 connect the chamber A with the other alternate spaces which face the orifices of the spinneret.

It will appear from a study of the arrangement of Figures 1 to 3, that if two different spinning materials or solutions are supplied by pipes 6 and 7, the material or solution immediately back of the spinneret face would be more or less stratified into alternating layers of the two types of spinning materials, one of the types being found in the spaces between the ribs 11 facing the spinneret orifices and the other type being found in the spaces between ribs 11 which face blank spaces of the spinneret face. Since both pumps force the spinning materials or solutions to find egress, the material or solution in the spaces between partitions 11 which face blank spaces of the spinneret face must flow through the spinneret orifices on either side of the spinning material or solution flowing through the spaces between the ribs 11 facing the spinneret orifices. Such flow gives rise to filament cross-sections such as those shown in Figure 8. If the pump associated with pipe 7 is operated at greater volumetric speed than that connected with pipe 6, the lateral portions of filament forming material completely envelop the central

portion as shown in Figure 8a. Where the pump speeds are more nearly equal, a cross-section of filament similar to Figure 8b is obtained, while if the pump associated with pipe 7 is operated at considerably lower volumetric output than that associated with pipe 6, the filament structure of Figure 8c is obtained. The cross-section can also be controlled by selection of spinning materials. For example, in the case of two viscoses, if the intermediate viscose shrinks more rapidly in setting up, than the outer viscose, the cross-section of Figure 8a is obtained, whereas a reversal of shrinkage characteristics results in the cross-section of Figure 8c. Again, control can be effected by altering both pump speeds and viscose shrinkage characteristics. Although the boundaries between the components of the filaments are shown distinctly in the drawing, there may be some intermingling of the different components on either side of the boundaries.

The extrusion device of this invention may be used for wet or dry spinning or for spinning molten materials. The two spinning materials may be solutions which may contain the same filament-forming substance in solution but differ in the kind of solvent or the concentration of the filament-forming substance. The spinning materials may be polymeric substances which differ in their degree of polymerization or degradation; in the case of cellulose or its derivatives, the two solutions can be produced from celluloses of different origin, for example one from cotton linters and the other from wood pulp. In the case of spinning solutions which undergo a ripening process, such as viscose, differences of degree of ripeness may be the sole difference or one of several differences (which may include also cellulose content, sodium hydroxide content, carbon disulfide content) between the spinning solutions.

The two spinning materials may comprise the same or different spinning substances, but differ in that one of the two contains incorporated therein, either suspended therein or dispersed therein, such as by true or colloidal solution or by emulsification, at least one substance which is not of itself a filament-forming substance. Alternatively, both spinning materials can contain one or more of such additions in different concentrations. Such additions can be solid, liquid or gaseous, for example pigments, roughening agents, softening agents, agents for improving the feel, fats, oils, soaps, resins, dyestuffs, fungicides, medicinal substances, phosphorescent substances, and substances which can react chemically with the spinning substance in the solution or during the precipitation. In particular, those additions which are used to modify the properties of the filaments and have hitherto involved unavoidable disadvantages when applied to homogeneous fibers can be restricted to that zone of the filament where they are desired. For example, pigments and delustrants which are introduced into the spinning mass for the purpose of roughening the surface of the filament, or of coloring or dulling the filament, cause a sensible decrease in the strength. By the new process, such substances, which can fulfil their purpose when disposed only at the surface of the filament, need be introduced only into the spinning material or solution for forming the outer envelope of Figure 8a, while the core remains undiluted by such additions and, therefore, maintains its normal strength.

When the process is carried out with two spinning solutions which contain different spinning

substances in solution, the two spinning substances can be chemically related, as, for example, two different cellulose esters, or a cellulose ester and a cellulose ether, or two different albuminous substances. Two spinning substances may, however, be used which belong to quite different classes of bodies, such as cellulose and an albuminous substance, or a cellulose ester or ether and an artificial resin or rubber produced by polymerization. The only limitation is that the two spinning materials do not mutually coagulate each other and are coagulatable by a common coagulating medium. According to whether one kind of spinning substance forms the core or intermediate portion and another kind the sheath or lateral portions of the filaments, or vice versa, filaments of different properties can be obtained from the same substances. By using two spinning materials which shrink to a different extent during precipitation, drying or after-treatment, there may be obtained, for example, strongly crimped threads. Also, one or both spinning materials or solutions may consist of or comprise mixtures of two or more filament-forming substances insofar as this is permitted by the compatibility of the particular substances.

Various effects may be obtained by enclosing a pigmented or dyed core by an uncolored sheath, or one which is colored but not so deeply as to prevent the core from exerting an influence on the appearance of the filament. By sandwiching a colorless or lightly colored component between lateral components intensely dyed or heavily pigmented to form structures having cross-sections similar to Figures 8b and 8c, or by reversing the disposition of the lightly and densely colored components respectively, novel and interesting effects are obtained, and such effects are accentuated when the two components are made of materials having different shrinkages, and are subsequently differentially shrunk to effect crimping thereof.

Further modifications may be obtained by changing the partition 12 from a simple transverse rib to a partition 12a of Y-shape (Figure 2a), and providing another pipe connection similar to 6 and 7 for supplying a third spinning material or solution to the third chamber Y thus provided. In that case, the central one of the spaces between the several partitions 11 is connected to the third chamber Y receiving the third spinning material or solution by a suitable passage 17y similar to the central passage 17 shown in Figure 2. In such an arrangement, the filaments would be composed of three filament-forming materials arranged similarly to the layers of Figures 8a, 8b and 8c, but with one of the laterally disposed materials of different composition than the other lateral member. This arrangement is illustrated in Figures 9a, 9b, 9c. This arrangement may be of particular advantage to form crimped filaments by associating a plurality of filament-forming materials at least two of which show different shrinkage characteristics, particularly after stretching, and subsequently crimping them by taking advantage of these characteristics.

Another modification is illustrated in Figure 3a in which the construction of the extrusion device is the same as in Figures 1 to 3, the only difference being that the strips of spinneret face opposed to the regions between partitions 11 are all occupied by orifices 16a, each strip being provided with a single row thereof. One set of alternate 75 regions in this embodiment is supplied with a fill-

ament-forming material in excess of the proportion supplied to the other regions relative to the total orifice cross-sectional area opposed to the respective sets of regions, thereby forcing the excess to produce composite filaments in either orifices 16 or 16a depending upon which regions are supplied with the excess that must flow into the other regions. There is thus produced a mixture of filaments, some formed of a single material and others formed of two or three materials depending upon whether the distributing system of Figure 2 or 2a is used. If the system of Figure 2a is used, filaments proceeding from the rows 16a can be made of a single material but those from the central row 16a will be of a different material than those from the outer rows 16a, and the rows 16 will produce filaments of the type shown in 9a, 9b, or 9c. The orifices may be regularly or irregularly disposed in that set of the alternate strips opposed to the regions supplied with the relatively greater amount of spinning material, and some of such orifices may extend partially or completely into the adjoining regions. The orifices in the several regions may be of various sizes to produce simultaneously different denier filaments from a single material and/or different denier filaments of composite character.

Further modifications can be obtained by utilizing a three-material distributor, such as that of Figure 2a with an orifice pattern such as that illustratively shown in Figure 3b. As shown, there are three rows of orifices 16a and two intervening rows of orifices 16 opposed to the regions between the partitions 11 as in Figure 3a. But in addition, there are two rows of orifices 16b approximately in alignment with the edges of the partitions. These rows of orifices 16b may be offset somewhat from the alignment shown without changing the results. The chamber Y of Figure 2a supplies filament-forming material to the central region between partitions 11 opposed to the central row of orifices 16a; chamber A, a second material, to adjacent regions opposed to orifice 16; and chamber B, a third material to the outer regions opposed to outer rows of orifices 16a. The proportions of the three materials relative to the total orifice area opposed to the regions supplied with the material can be readily controlled to produce various combinations of filaments. For example, the outer rows of orifices 16a will issue filaments formed solely of the third material and the orifices 16 will issue filaments formed solely of the second material, while orifices 16b will issue dual-component filaments composed of the second and third material joined side by side the entire length thereof and the central orifices 16a will issue triple-component filaments (as in Figure 8a, 8b or 8c) formed of the first and second materials. By increasing the supplies of the first and third materials relative to the second, however, the system can be made to produce the following mixture of filaments: filaments solely of first material from inside row of orifices 16a, filaments solely of third material from outside rows of orifices 16a and also from orifices 16b, while triple-component filaments formed of all three materials (as in Figure 9a, 9b or 9c) will issue from orifices 16. It will thus be seen that numerous mixtures and combinations of filaments can be obtained directly from a single spinneret without difficulty. Further variations can be made by changing the groups of regions between partitions 11 supplied by the several materials.

Figures 4 to 7 show a modification of the ex-

trusion device in which the partitioning means within the space back of the spinneret face is arranged to co-operate with a spinneret having concentric groups of orifices, such as circular rows of orifices. In this arrangement, the space immediately back of the spinneret face is divided by a plurality of concentric partitions 21 (four being shown, though any number may be used) into concentric annular chamber C<sub>1</sub>, C<sub>2</sub>, C<sub>3</sub> and C<sub>4</sub> about a central chamber C. These partitions 21 may extend from a transverse plate 22 secured in or integrally formed in a sleeve 23 fitting within the walls of the spinneret 2 and the recess 14 on the supply head 3. In the space back of the plate 22, there is disposed a distributor member having a transverse plate 24 from which the concentric partitions 25 extend into contact with plate 22. A transverse rib or partition 26 divides the space back of the plate 24 into two compartments or chambers A and B. A locating pin 27 extends from a bore in one of the walls 28 extending back of the plate 24 through a slot in sleeve 23 to a slot 29 in the supply head 3. This locating pin 27 is arranged so that the passages 8 and 9 are each associated with only one of the compartments A and B respectively on either side of the rib 26. The passages 30 join compartment B with alternate regions or chambers between the concentric partitions 25, while passages 31 connect the compartment A with the other annular regions or chambers (including the central region) between partitions 25. Passages 32 connect the corresponding regions and chambers in front of and in back of plate 22. The orifices of the spinneret are arranged to face alternate annular regions or chambers between the annular partitions 21, namely C<sub>1</sub> and C<sub>3</sub>, thus leaving blank the portions of the spinneret face opposite the intervening chambers C, C<sub>2</sub> and C<sub>4</sub> between partitions 21.

The operation of the device of Figures 4 to 7 is analogous to that of Figures 1 to 3, the spinning materials or solutions immediately behind the spinneret face being arranged as concentric strata instead of the parallel linear strata of Figures 1 to 3. As in Figure 2a, the partition 26 may similarly be made of Y-shape and an additional spinning material feed pipe similar to 6 and 7 may be provided and connected with the third compartment thus provided by the Y-shape of partition 26. In such event, the third compartment may be connected with a separate region or chamber between the partitions 25 by passages similar to 30 and 31, so that the spinning materials will alternate in sequence to provide filaments similar to those of Figure 9. Thus the third spinning material may be directed into the chamber C<sub>2</sub>, leaving the other two materials to follow the same channels as shown in the drawing. Also, additional orifices may be supplied to the blank strips of the spinneret shown in the drawing, to form combinations analogous to those illustrated in Figures 3a and 3b.

The following examples are illustrative of the invention:

#### Example I

Equal volumetric amounts of two different types of viscose solutions were spun, through a form of apparatus similar to that described above and shown in Figure 4, into a spinning bath containing 10% sulfuric acid, 2% zinc sulfate and 19% sodium sulfate at a temperature of 45° C. One of the types of viscose solution was made from wood pulp using 30% carbon disulfide based

on the air dry weight of the pulp and contained 7½% cellulose and 6½% sodium hydroxide. This viscose was aged for 100 hours and had a common salt point of 1.9. The other type of viscose solution was made from cotton pulp using 44% carbon disulfide based on the air dry weight of the pulp and contained 7½% cellulose and 8% sodium hydroxide. To this viscose was added 6% finely ground titanium dioxide based on the weight of cellulose present. This viscose was aged for 48 hours and had a common salt point of 5.5. The young viscose containing titanium dioxide was allowed to pass through the apparatus, so as to enter the blank spaces of the spinneret face C, C<sub>2</sub> and C<sub>4</sub>. The other viscose entered the alternate spaces facing the spinneret orifices C<sub>1</sub> and C<sub>3</sub>. Owing to the more rapid setting up or shrinkage rate of the older viscose the titanium dioxide containing viscose almost completely surrounded the other viscose to give a cross-section approaching closely that shown in Figure 8a. The resulting filaments which were of 5 denier had a dull delustered appearance owing to the presence of the titanium dioxide on the outside sheath of the filament.

*Example II*

Two different types of viscose solution were prepared and spun exactly the same as in Example I, with the exception that the titanium dioxide was added to the older viscose made from wood pulp instead of being added to the younger viscose. The cross-section which was of the type shown in Figure 8a contained the titanium dioxide viscose surrounded by the other viscose, which imparted to the filaments a glossy delustered appearance owing to the presence of the delustrant in the core of the filament.

*Example III*

Two different types of viscose solution were prepared and spun exactly as in Example I, with the exception that the young titanium dioxide containing viscose was allowed to pass through the apparatus so as to enter the spaces C<sub>1</sub> and C<sub>3</sub> facing spinneret orifices, and the old viscose to enter the face blank spaces C, C<sub>2</sub> and C<sub>4</sub>. The resulting cross-section was of the type illustrated in Figure 8c with the titanium dioxide containing viscose only partially surrounding the other viscose.

It is to be understood that changes and variations may be made without departing from the spirit and scope of the invention as defined by the appended claims.

We claim:

1. A filament extrusion device comprising a spinneret having a row comprising at least two orifices, partition means for dividing the space back of the spinneret face into at least three substantially separate regions arranged side by side, one of said regions being disposed opposite the row of orifices and communicating with the two adjacent regions just behind the spinneret face along spaced planes in the vicinity of, but laterally offset on opposite sides from, the row of orifices, and conduit means having channel systems associated with each of the separate regions for introducing filament-forming material of at least two different kinds so that the materials supplied to immediately adjacent regions are different from each other and each material flows separately into at least one of said regions.

2. A filament extrusion device comprising a spinneret having a row comprising at least two

orifices, partition means for dividing the space back of the spinneret face into at least three substantially separate regions arranged side by side, one of said regions being disposed opposite the row of orifices and communicating with the two adjacent regions just behind the spinneret face along spaced planes in the vicinity of, but laterally offset on opposite sides from, the row of orifices, at least one other orifice disposed outside of said row in a strip of the spinneret face laterally offset therefrom, and conduit means having channel systems associated with each of the separate regions for introducing filament-forming material of at least two different kinds so that the materials supplied to immediately adjacent regions are different from each other and each material flows separately into at least one of said regions, whereby said row of orifices may receive material simultaneously from three adjacent regions and said other orifice may receive material only from a single one of the regions.

3. A filament extrusion device comprising a spinneret having a row comprising at least two orifices, partition means for dividing the space back of the spinneret face into at least three substantially separate regions arranged side by side, one of said regions being disposed opposite the row of orifices and communicating with the two adjacent regions just behind the spinneret face along spaced planes in the vicinity of and parallel to, but laterally offset on opposite sides from, the row of orifices, at least one other orifice disposed outside of said row in a strip of the spinneret face adjacent said row, but laterally offset therefrom, and conduit means having channel systems associated with each of the separate regions for introducing filament-forming material of at least two different kinds so that the materials supplied to immediately adjacent regions are different from each other and each material flows separately into at least one of said regions, whereby said row of orifices may receive material simultaneously from three adjacent regions and said other orifice may receive material only from a single one of the regions.

4. A filament extrusion device comprising a spinneret having a row comprising at least two orifices, partition means for dividing the space back of the spinneret face into at least three substantially separate regions arranged side by side, one of said regions being disposed opposite the row of orifices and communicating with the two adjacent regions just behind the spinneret face along spaced planes in the vicinity of, but laterally offset on opposite sides from, the row of orifices, at least one other orifice disposed outside of said row in a strip of the spinneret face laterally offset therefrom and disposed opposite one of the regions immediately adjacent that region opposite said row, and conduit means having channel systems associated with each of the separate regions for introducing filament-forming material of at least two different kinds so that the materials supplied to immediately adjacent regions are different from each other and each material flows separately into at least one of said regions, whereby said row of orifices may receive material simultaneously from three adjacent regions and said other orifice may receive material only from a single one of the regions.

5. A filament extrusion device comprising a spinneret having a row comprising at least two orifices, partition means for dividing the space back of the spinneret face into at least four substantially separate regions arranged side by side,

one of said regions being disposed opposite the row of orifices and communicating with the two adjacent regions just behind the spinneret face along spaced planes in the vicinity of, but laterally offset on opposite sides from, the row of orifices, at least one other orifice disposed outside of the row in proximity to the plane of communication between two adjacent regions other than that opposed to the row of orifices, and conduit means having channel systems associated with each of the separate regions for introducing filament-forming material of at least three different kinds so that the materials supplied to immediately adjacent regions are different from each other and each material flows separately into at least one of said regions, whereby said row of orifices may receive material simultaneously from three adjacent regions and said other orifice may receive material only from two adjacent regions.

6. A filament extrusion device comprising a spinneret having a row comprising at least two orifices, partition means for dividing the space back of the spinneret face into at least four substantially separate regions arranged side by side, one of said regions being disposed opposite the row of orifices and communicating with the two adjacent regions just behind the spinneret face along spaced planes in the vicinity of, but laterally offset on opposite sides from, the row of orifices, at least one other orifice disposed outside of said row in a strip of the spinneret face laterally offset therefrom, at least one other orifice disposed outside of the row in proximity to the plane of communication between two adjacent regions other than that opposed to the row of orifices, and conduit means having channel systems associated with each of the separate regions for introducing filament-forming material of at least three different kinds so that the materials supplied to immediately adjacent regions are different from each other and each material flows separately into at least one of said regions, whereby said row of orifices may receive material simultaneously from three adjacent regions, said first-mentioned other orifice may receive material from a single one of the regions, and the last-mentioned other orifice may receive material from two adjacent regions.

7. A filament extrusion device comprising a spinneret having a plurality of rows of orifices, partitions for dividing the space back of the spinneret face into at least three substantially separate regions arranged side by side, each region being disposed opposite at least one of said rows of orifices and communicating with each adjacent region just behind the spinneret face along spaced planes projecting from the edge of the partitions of the spinneret face, and conduit means having channel systems associated with each of the separate regions for introducing filament-forming material of at least two different kinds so that the materials supplied to immediately adjacent regions are different from each other and each material flows separately into at least one of said regions.

8. A filament extrusion device comprising a spinneret having a plurality of rows of orifices, partitions for dividing the space back of the spinneret face into at least three substantially separate regions arranged side by side, each region being disposed opposite at least one of said rows of orifices and communicating with each adjacent region just behind the spinneret face along spaced planes projecting from the edge of the partitions to the spinneret face, and con-

duit means having channel systems associated with each of the separate regions for introducing filament-forming material of at least two different kinds so that the materials supplied to immediately adjacent regions are different from each other and each material flows separately into at least one of said regions, and means for predeterminedly controlling the relative rates of flow of said different materials so that at least one of said rows of orifices receives material simultaneously from three adjacent regions and at least one other of said rows receives material from a region other than that opposite those orifices receiving material simultaneously from three adjacent regions.

9. A filament extrusion device comprising a spinneret having a plurality of rows of orifices, partitions for dividing the space back of the spinneret face into at least four substantially separate regions arranged side by side, each region being disposed opposite at least one of said rows of orifices and communicating with each adjacent region just behind the spinneret face along spaced planes projecting from the edge of the partitions to the spinneret face, at least one other of said rows of orifices being disposed adjacent the plane of communication between two adjacent regions, and conduit means having channel systems associated with each of the separate regions for introducing filament-forming material of at least three different kinds so that the materials supplied to immediately adjacent regions are different from each other and each material flows separately into at least one of said regions.

35 10. A filament extrusion device comprising a spinneret having a plurality of rows of orifices, partitions for dividing the space back of the spinneret face into at least four substantially separate regions arranged side by side, each region being disposed opposite at least one of said rows of orifices and communicating with each adjacent region just behind the spinneret face along spaced planes projecting from the edge of the partitions to the spinneret face, at least one other of said rows of orifices being disposed adjacent the plane of communication between two adjacent regions, and conduit means having channel systems associated with each of the separate regions for introducing filament-forming material of at least three different kinds so that the materials supplied to immediately adjacent regions are different from each other and each material flows separately into at least one of said regions, and means for predeterminedly controlling the relative rates of flow of said different materials so that at least one of said rows of orifices receives material simultaneously from three adjacent regions and at least one other of said first-mentioned rows receives material from a region other than that opposite those orifices receiving material simultaneously from three adjacent regions, and so that said other row of orifices disposed adjacent the plane of communication of two adjacent regions receives material from the respective adjacent regions.

11. A filament extrusion device comprising a spinneret having a row comprising at least two orifices and a blank strip disposed on each side of the row, partition means for dividing the space back of the spinneret face into at least three substantially separate regions arranged side by side, one of said regions being disposed opposite the row of orifices and communicating with the two adjacent regions just behind the spinneret face along spaced planes in the vicinity of, but

## 11

laterally offset on opposite sides from, the row of orifices, said two adjacent regions being disposed opposite said blank strips, and conduit means having channel systems associated with each of the separate regions for introducing filament-forming material of at least two different kinds so that the materials supplied to immediately adjacent regions are different from each other and each material flows separately into at least one of said regions.

12. A filament extrusion device comprising a spinneret having a plurality of groups of orifices separated by intervening blank strips of the spinneret face, partition means for dividing the space back of the spinneret face into a plurality of substantially separate regions arranged side by side, each two adjacent regions communicating with each other just behind the spinneret face along a plurality of pairs of spaced planes, the planes of each pair being disposed in the vicinity of, but laterally offset on opposite sides from, one of the groups of the orifices, alternate ones of the regions being disposed generally opposite the groups of orifices and the intervening regions being disposed opposite the blank portions of the spinneret face, and conduit means having separate channel systems associated with each of the separate regions for introducing filament-forming material of at least two different kinds so that each of such materials flows separately into regularly spaced ones of the regions.

13. A filament extrusion device comprising a spinneret having a plurality of rows of orifices separated by intervening blank strips of the spinneret face, a plurality of partitions generally parallel to the rows dividing the space back of the spinneret into regions, alternate ones of such regions being in approximate alignment with the orifices and intervening regions facing the blank strips of the spinneret, and a plurality of conduit means each having a separate channel system associated with a separate group of regularly spaced regions for introducing filament-forming material thereto.

## 12

14. A filament extrusion device comprising a spinneret having a plurality of rows of orifices separated by intervening blank strips of the spinneret face, a plurality of partitions generally parallel to the rows dividing the space back of the spinneret into regions, alternate ones of such regions being in approximate alignment with the orifices and intervening regions with faced with the blank strips of the spinneret, and two conduit means each having a separate channel system associated with a separate group of regularly spaced regions for introducing filament-forming material thereto.

15. A filament extrusion device comprising a spinneret having a plurality of annular groups of orifices separated by intervening blank strips of the spinneret face, a plurality of annular partitions dividing the space back of the spinneret into concentric regions, alternate ones of such regions being in approximate alignment with the orifices and intervening regions facing the blank strips of the spinneret, and a plurality of conduit means each having a separate channel system associated with a separate group of regularly spaced regions for introducing filament-forming material thereto.

16. A filament extrusion device comprising a spinneret having a plurality of annular groups of orifices separated by intervening annular blank strips of the spinneret face, a plurality of annular partitions dividing the space back of the spinneret into concentric regions, alternate ones of such regions being in approximate alignment with the orifices and intervening regions facing the blank strips of the spinneret, and two conduit means each having a separate channel system associated with a separate group of regularly spaced regions for introducing filament-forming material thereto.

WAYNE A. SISSON.  
WESLEY L. WEBB.